

## UNITED STATES PATENT OFFICE

2,615,843

## OIL COMPOSITIONS CONTAINING STABILIZED COPOLYMER ESTER-TYPE POUR POINT DEPRESSANTS

John J. Giammaria, Woodbury, N. J., assignor to Socony-Vacuum Oil Company, Incorporated, a corporation of New York

No Drawing. Application August 31, 1951,  
Serial No. 244,716

9 Claims. (Cl. 252—33.4)

1

This invention relates to lubricating oil compositions. More particularly, the invention relates to lubricating oil compositions containing a pour point depressant of the copolymer ester-type and a basic sulfonate-type detergent.

As is well known in the lubricating art, the various characteristics of mineral lubricating oils may be enhanced by the addition thereto of relatively small amounts of various chemical agents designed to effect certain specific improvements therein. Thus, addition agents are known which have the ability to fortify the oil against oxidation, improve its detergent action, increase its load-carrying ability, improve its viscosity, depress the pour point of the oil, etc. These chemical agents are known in the art as antioxidants, detergents, extreme pressure agents, V. I. (viscosity index) improvers and pour point depressants.

As is further known, it is the practice in the art to add to mineral lubricating oils not just one additive, but combinations of additives whereby more than one characteristic of the oil is improved. The present invention is concerned with an oil containing such a combination of additives, viz., (a) a pour point depressant of the copolymer ester-type and (b) a basic sulfonate-type detergent. In the use of these two types of additives in combination in oil, it was found that the detergent exhibited a deleterious effect on the pour point depressant, at the concentrations of additives normally used, so that the latter's ability to lower the pour point of the oil was substantially destroyed. For example, 0.025 weight per cent of an esterified copolymer of the character herein contemplated lowered the A. S. T. M. pour point of a base oil from +20° F. to -15° F. but, upon adding a basic sulfonate type of detergent to this blend, the A. S. T. M. pour point was raised to +10° F. Due to the incompatibility thus exhibited by the additives, the use of the copolymer ester-type pour depressants in combination with the basic sulfonate-type detergent was, of course, not feasible. This posed a serious problem since the copolymer esters are an extremely effective and highly desirable type of pour depressant and the basic sulfonates are likewise exceptionally good detergents and the use of the two in combination in an oil was, therefore, highly desirable.

It is the object of this invention to provide a

2

process whereby copolymer ester-type pour point depressants can be stabilized for use in oil compositions containing basic sulfonate detergents and also to provide oil compositions containing such stabilized pour point depressants and detergents.

In accordance with the present invention, it has now been found that pour point depressants of the copolymer ester-type may be successfully stabilized for use with basic sulfonate detergents by reacting the pour depressant with a small amount of a primary amine. The procedure involves adding a minor amount, from about 2 to about 10 per cent by weight, generally 3 to 4 per cent, of the primary amine to the pour depressant and heating to a temperature of from about 150° C. to about 200° C. This temperature is maintained for about ½ to 2 hours. The reaction may be carried out with or without a solvent. Suitable solvents include xylene, naphtha or other high-boiling hydrocarbons. The solvent is subsequently removed by distillation. A mineral oil may also be used as a solvent for the reaction in which case it need not be removed, but the product, being thus obtained in the form of an oil concentrate, may be added directly to the lubricating oil sought to be improved in pour point character. When a solvent is not used, it is preferred to first heat the pour depressant to about 100° C. and then add the amine in order to avoid any thickening or gelation which may otherwise occur.

Any primary amine of the aliphatic, aromatic, cycloaliphatic or heterocyclic series may be used in the invention. In general, aliphatic, straight-chain, primary amines having from 1 to about 18 carbon atoms are preferred, while those having 12 to 18 carbon atoms are particularly preferred.

Typical of the amines which may be used in the invention are the following: (a) aliphatic amines, such as methylamine, ethylamine, propylamine, butylamine, hexylamine, octylamine, decylamine, tetradecylamine, hexadecylamine and octadecylamine; (b) cycloaliphatic amines, such as cyclohexylamine and cyclopropylamine; (c) aromatic amines, such as aniline, naphthylamine, toluidine and anisidine; and (d) heterocyclic amines, such as 2-aminopyridine, 2-aminothiophene and 2-aminofuran.

The copolymer ester-type pour depressants

particularly contemplated herein are those prepared by copolymerizing maleic anhydride with styrene and then esterifying the copolymer product with a primary, normal, aliphatic alcohol having from 12 to 14 carbon atoms, or a mixture of alcohols having from 10 to 18 carbon atoms and an average of 12 to 14 carbon atoms per molecule. The copolymers are prepared by reacting maleic anhydride and styrene in approximately equimolar quantities in the presence of a peroxide polymerization catalyst, such as benzoyl peroxide, at a temperature of from about 50° C. to about 150° C. An excess of styrene may be used in order to insure complete reaction of the maleic anhydride, the excess styrene being conveniently removed from the reaction mixture by distillation after the reaction is complete. The reaction is generally complete in from about 1 to about 5 hours. This reaction may be conducted in a suitable solvent, such as xylene, toluene, dioxane, or the like.

The esters of the copolymers are readily prepared by reacting the copolymer and a suitable alcohol under ordinary esterification conditions. For example, the reactants may be heated at xylene reflux temperature in the presence of concentrated sulfuric acid, or p-toluene sulfonic acid, as a catalyst. As aforesaid, suitable alcohols for this purpose are the primary, normal, saturated, monohydric, aliphatic alcohols of from 12 to 14 carbon atoms, such as lauryl alcohol or tetradecyl alcohol, or a mixture of alcohols having from about 10 to about 18 carbon atoms and an average of 12 to 14 carbon atoms per molecule. Typical of suitable alcohol mixtures are two mixtures of alcohols manufactured and marketed by E. I. du Pont de Nemours Company under the trade-names "Lorol-5" and "Lorol-B". These mixtures contain normal, aliphatic, saturated, monohydric aliphatic alcohols containing 10 to 18 carbon atoms in approximately the following proportions:

|                                   | "Lorol-B" | "Lorol-5" |
|-----------------------------------|-----------|-----------|
| C <sub>10</sub> .....percent..... | 2.5       | 2.8       |
| C <sub>12</sub> .....do.....      | 55.0      | 61.0      |
| C <sub>14</sub> .....do.....      | 20.5      | 21.0      |
| C <sub>16</sub> .....do.....      | 9.0       | 11.0      |
| C <sub>18</sub> .....do.....      | 13.0      | 2.2       |
| Ave. No. C Atoms.....             | 13.5      | 12.7      |

Although the esters prepared from maleic anhydride-styrene copolymers are particularly contemplated herein, the invention may be applied to various other copolymer ester-type pour depressants, such as the esters of other vinyl or allyl compounds copolymerized with maleic anhydride. For example, the invention is applicable where the pour point depressant is a 1-olefin-maleic anhydride copolymer ester, a vinyl-ester-maleic anhydride copolymer ester, a vinyl-ether-maleic anhydride copolymer ester, or the like. Ester-type copolymers to which the invention is applicable are described in detail in copending applications, Serial No. 744,802, Serial No. 756,316 and Serial No. 77,288 of the present inventor, and Serial No. 736,106, now Patent No. 2,570,846 issued October 9, 1951 and Serial No. 739,652 of Ferdinand P. Otto et al.

The basic sulfonate detergents contemplated herein are particularly those obtained from aromatic hydrocarbons, substituted aromatic hydrocarbons or aromatic petroleum fractions and a sulfonating agent, such as strong sulfuric acid,

oleum, chlorosulfonic acid and the like, the petroleum-type sulfonates being particularly preferred. Synthetic types of sulfonates may also be used, such as the basic metal salts of sulfonic acids or wax-substituted benzene and naphthalene, wherein the wax substituent is a long-chain aliphatic hydrocarbon obtained from petroleum and having at least about 18 carbon atoms and generally an average of about 24 carbon atoms per molecule.

The basic salts particularly contemplated herein are those of the metals calcium, barium, strontium and magnesium. The basic salt is produced by reacting the sulfonic acid with an excess of the metal hydroxide over that which would be required to neutralize it or any occluded sulfuric acid which might be present therein.

The following examples and tests will serve to illustrate the utility of the present invention.

#### EXAMPLE A

##### Basic barium petroleum sulfonate

A basic sulfonate detergent was prepared as follows: A Mid-Continent-type residual oil was sulfonated by slowly adding 300 parts of 103 per cent H<sub>2</sub>SO<sub>4</sub> to 1000 parts of oil at 100-140° F. Sixty parts of H<sub>2</sub>O were added and the temperature was maintained at 160-170° F. for 24 hours. The upper sour oil layer was drawn off and air blown to remove dissolved SO<sub>2</sub>.

Ninety-two parts of BaO were slaked with 270 parts of water in a separate reactor. At 170° F., 1040 parts of sour oil were added. The temperature was slowly raised to 200° F. and the product was dehydrated by air blowing at this temperature. The final product was obtained by filtering under pressure at 200° F.

#### EXAMPLE I

##### Mixed alcohol ester of styrene-maleic anhydride copolymer

(a) A copolymer ester-type pour depressant was prepared as follows:

Sixty parts of styrene and 40 parts of maleic anhydride were dissolved in 1000 parts of toluene by heating to 75° C. One part of benzoyl peroxide was added and the temperature was raised to 95° C. where the copolymerization reaction started. The styrene-maleic anhydride copolymer precipitated as the reaction progressed. The mixture was heated at reflux for about 1/2 hour. It was then cooled to 100° C. and 177.2 parts of a mixture comprising 75 per cent by weight of "Lorol-5" and 25 per cent by weight of octadecanol-1 were added. One and one-half parts of concentrated H<sub>2</sub>SO<sub>4</sub> were added and the mixture heated at reflux for 1 hour. The water formed during the esterification of the copolymer was collected in a Dean-Stark moisture trap. The solvent was gradually distilled from the reaction mixture and the temperature was finally raised to 175° C. to complete the esterification.

(b) The copolymer ester from (a) was diluted with sufficient mineral oil to make a 40 per cent (by weight) blend of the copolymer ester to facilitate handling. Two parts of n-dodecylamine were added to 50 parts of the oil solution of the pour depressant at room temperature. The solution became quite viscous whereupon 50 parts of xylene were added as a diluent. The temperature was gradually raised to 175° C. and the xylene removed by distillation. Heating was continued at 175° C. for 1 hour. On cooling to room tem-

perature, the product remained fluid and showed no signs of gelling on subsequent storage.

EXAMPLE II

Two parts of n-octadecylamine were added to 50 parts of the copolymer ester described in Example I(a) and the mixture was heated at 175° C. for 1 hour.

EXAMPLE III

Two parts of cyclohexylamine were added to 50 parts of the copolymer ester described in Example I(a) at 100° C. Heating was continued to 175° C. and maintained for 1 hour.

EXAMPLE IV

Two parts of aniline were added to 50 parts of the copolymer ester described in Example I(a) at 100° C. The temperature was then raised to 175° C. and held for 1 hour. The mixture was finally heated to 185° C. under reduced pressure to remove unreacted aniline.

EXAMPLE V

This example was the same as Example I(a), but n-butylamine was substituted for n-dodecylamine.

*Stabilization of pour point depressant*

The test results shown in Table I illustrate the improvement in pour point lowering effect obtained with the amine-modified pour depressant when used in conjunction with a basic sulfonate detergent similar to that described in Example A, namely, a basic barium salt of a petroleum sulfonic acid. The test oil was a solvent-refined, Mid-Continent type base oil having a kinematic viscosity of 6.37 centistokes at 210° F. and an A. S. T. M. pour point of +20° F. It is seen from these data that the effectiveness of the untreated copolymer ester is greatly reduced when the basic detergent is added to the blend while the amine-modified products remain substantially unchanged in their effectiveness in the presence of the detergent.

TABLE I

| Compound(s) Blended in Oil            | A. S. T. M.<br>Pour Point, °F. |
|---------------------------------------|--------------------------------|
| None                                  | +20                            |
| .025% Detergent                       | -15                            |
| .025% of Example I(a)+2.75% Detergent | +15                            |
| .025% of Example I(b)+2.75% Detergent | +10                            |
| .025% of Example II+2.75% Detergent   | -15                            |
| .025% of Example III+2.75% Detergent  | -10                            |
| .025% of Example IV+2.75% Detergent   | -10                            |
| .025% of Example V+2.75% Detergent    | -15                            |

The amounts of stabilized, esterified copolymer pour depressant to be used in the oil compositions contemplated herein, along with the basic sulfonate detergent, range from about 0.01 weight per cent to about 0.5 weight per cent and particularly from 0.025 weight per cent to 0.05 weight per cent. The basic sulfonate detergent, on the other hand, may be added to the oil in amounts ranging from about 1 to about 10 per cent by weight and preferably from about 2 to 3 per cent.

Other addition agents may also be used in the oil along with the additives herein contemplated. The additive combinations herein disclosed may be prepared in the form of oil concentrates, if desired, to provide an additive base which is readily soluble in lubricating oils.

Although the principle of the invention has been illustrated by means of a particular stabilized copolymer-ester and a specific basic sul-

fonate detergent, it is intended that the invention not be limited in any way thereby, but only as defined in the appended claims.

What is claimed is:

1. A mineral lubricating oil containing (a) a minor amount, sufficient to improve the detergent character of said oil, of a basic metal sulfonate and (b) a minor amount, sufficient to depress the pour point of said oil of an esterified copolymer which has been stabilized against the deleterious effect normally exerted on said esterified copolymer by the basic metal sulfonate in the oil, which effect reduces the ability of said esterified copolymer to lower the pour point of said oil; said esterified copolymer having been formed by reacting a vinyl compound, selected from the group consisting of styrene, 1-olefins, vinyl esters and vinyl ethers, with maleic anhydride in about equimolar quantities and then esterifying the copolymer thus formed with an alcohol material selected from the group consisting of primary, normal, saturated, aliphatic alcohols having from 12 to 14 carbon atoms and a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of a primary amine at a temperature of from about 125° C. to about 200° C., for a period of from about 1 to about 5 hours.
2. A mineral lubricating oil containing (a) a minor amount, sufficient to improve the detergent character of said oil, of a basic metal sulfonate and (b) a minor amount, sufficient to depress the pour point of said oil of an esterified copolymer which has been stabilized against the deleterious effect normally exerted on said esterified copolymer by the basic metal sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with an alcohol material selected from the group consisting of primary, normal, saturated, aliphatic alcohols having from 12 to 14 carbon atoms and a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of a primary amine at a temperature of from about 125° C. to about 200° C., for a period of from about 1 to about 5 hours.
3. A mineral lubricating oil containing (a) a minor amount, sufficient to improve the detergent character of said oil, of a basic metal petroleum sulfonate and (b) a minor amount, sufficient to depress the pour point of said oil of an esterified copolymer which has been stabilized against the deleterious effect normally exerted on said esterified copolymer by the basic metal petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with an alcohol material selected from the group consisting of primary, normal, saturated, aliphatic alcohols having from 12 to 14 carbon atoms and a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of a primary amine at a temperature of from about 125° C. to about 200° C., for a period of from about 1 to about 5 hours.

a mixture of primary, normal, saturated, aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of a primary amine at a temperature of from about 125° C. to about 200° C., for a period of from about 1 to about 5 hours.

4. A mineral lubricating oil containing (a) a minor amount, sufficient to improve the detergent character of said oil, of a basic barium petroleum sulfonate and (b) a minor amount, sufficient to depress the pour point of said oil of an esterified copolymer which has been stabilized against the deleterious effect normally exerted on said esterified copolymer by said basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with an alcohol material selected from the group consisting of primary, normal, saturated, aliphatic alcohols having from 12 to 14 carbon atoms and a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of a primary amine at a temperature of from about 125° C. to about 200° C., for a period of from about 1 to about 5 hours.

5. A mineral lubricating oil containing (a) a minor amount, sufficient to improve the detergent character of said oil, of a basic barium petroleum sulfonate and (b) a minor amount, sufficient to depress the pour point of said oil of an esterified copolymer which has been stabilized against the deleterious effect normally exerted on said esterified copolymer by the basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with a mixture of primary, normal, saturated, aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of n-octadecylamine at a temperature of from about 125° C. to about 200° C., for a period of from about 1 to about 5 hours.

6. A mineral lubricating oil containing (a) a minor amount, sufficient to improve the detergent character of said oil, of a basic barium petroleum sulfonate and (b) a minor amount, sufficient to depress the pour point of said oil of an esterified copolymer which has been stabilized against the deleterious effect normally exerted on said esterified copolymer by said basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with a mixture of primary, normal, saturated aliphatic alcohols having from 10 to 18 carbon

atoms and an average of from 12 to 14 carbon atoms per molecule; said esterified copolymer having been stabilized by reaction of said esterified copolymer with from about 1 to about 10 per cent by weight of n-butylamine at a temperature of from about 125° C. to about 200° C., for a period of from about 1 to about 5 hours.

7. A mineral lubricating oil containing (a) a minor amount, sufficient to improve the detergent character of said oil, of a basic barium petroleum sulfonate and (b) a minor amount, sufficient to depress the pour point of said oil of an esterified copolymer which has been stabilized against the deleterious effect normally exerted on said esterified copolymer by said basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of n-hexadecylamine at a temperature of from about 125° C. to about 200° C., for a period of from about 1 to about 5 hours.

8. A mineral lubricating oil containing (a) a minor amount, sufficient to improve the detergent character of said oil, of a basic barium petroleum sulfonate and (b) a minor amount, sufficient to depress the pour point of said oil of an esterified copolymer, stabilized against the deleterious effect normally exerted on said esterified copolymer by said basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of cyclohexylamine at a temperature of from about 125° C. to about 200° C., for a period of from about 1 to about 5 hours.

9. A mineral lubricating oil containing (a) a minor amount, sufficient to improve the detergent character of said oil, of a basic barium petroleum sulfonate and (b) a minor amount, sufficient to depress the pour point of said oil of an esterified copolymer which has been stabilized against the deleterious effect normally exerted on said esterified copolymer by said basic barium petroleum sulfonate in the oil, which effect reduces the ability of said esterified copolymer to lower the pour point of said oil; said esterified copolymer having been formed by reacting styrene with maleic anhydride in about equimolar quantities and then esterifying the copolymer thus formed with a mixture of primary, normal, saturated aliphatic alcohols having from 10 to 18 carbon atoms and an average of from 12 to 14 carbon atoms per molecule; said esterified copolymer having been stabilized by reaction of said esterified copolymer with from about 1 to about 10 per cent by weight of aniline at a temperature of from about 125° C. to about

200° C., for a period of from about 1 to about 5 hours.

JOHN J. GIAMMARIA.

**REFERENCES CITED**

The following references are of record in the file of this patent:

**UNITED STATES PATENTS**

| Number    | Name             | Date          | Number | Name      | Date |
|-----------|------------------|---------------|--------|-----------|------|
| 2,047,398 | Voss et al.      | July 14, 1936 | 10     | 2,397,454 |      |
| 2,168,535 | Nuesslein et al. | Aug. 8, 1939  |        | 2,478,015 |      |

| Number    | Name           | Date          |
|-----------|----------------|---------------|
| 2,200,429 | Perrin et al.  | May 14, 1940  |
| 2,301,356 | Arnold et al.  | Nov. 10, 1942 |
| 2,327,705 | Frolich et al. | Aug. 24, 1943 |
| 2,342,113 | Blair          | Feb. 22, 1944 |
| 2,366,517 | Gleason        | Jan. 2, 1945  |
| 2,370,943 | Dietrich       | Mar. 6, 1945  |
| 2,375,516 | Blair          | May 8, 1945   |
| 2,378,629 | Hanford        | June 19, 1945 |
|           | Woodward       | Mar. 26, 1946 |
|           | Rust           | Aug. 2, 1949  |